# EUROPEAN PATENT SPECIFICATION

(11) **EP 2 034 862 B1**
(45) Date of publication and mention of the grant of the patent: **21.10.2009**
(21) Application number: 07785879.3
(22) Date of filing: 02.07.2007
(51) Int. Cl.: A44B 18/00

(54) **RELEASABLE MECHANICAL FASTENER DEVICE**
LÖSBARES MECHANISCHES BEFESTIGUNGSELEMENT
DISPOSITIF D'ATTACHE MÉCANIQUE LIBÉRABLE

(30) Priority: 05.07.2006 IT MI20061300
(43) Date of publication of application: 18.03.2009
(73) Proprietor: Nuova Pansac S.p.A., 20124 Milano (IT)
(72) Inventor: LORI, Fabrizio, I-46030 Cerese di Virgilio (MN) (IT); BORTOLETTO, Graziano, I-31059 Zero Branco (TV) (IT)
(74) Representative: Premru, Rok
(86) International application number: PCT/EP2007/005822
(87) International publication number: WO 2008/003438

(56) References cited:
- EP-A1- 0 341 993
- EP-A2- 1 048 236
- EP-B1- 0 804 133
- US-A1- 2005 136 213

## Description

Disclosed herein is a releasable mechanical fastener device, which comprises two elements, such as two straps, which can be pressed together for mutual engagement and released by a tearing action.

The device disclosed below finds application, for instance, in the field of clothing and particularly of personal hygiene items, such as infant diapers and incontinence pads.

Fastener devices are known in the art - available with trade names such as Velcro ® and Microplast ® - which comprise a male member, with generally and/or substantially hook- or mushroom-shaped elements thereon, and a female member, with generally and/or substantially loop-shaped elements thereon, for mutual engagement.

Female straps are known to be formed, particularly, by attaching nonwoven fabrics having particular fiber arrangements to facilitate engagement to a support film, see for example EP 1 048 236 A.

Nevertheless, the use of female straps as a means for engagement of the hook elements of the male straps has certain drawbacks.

Prior art clothing and personal hygiene items, such as diapers and incontinence pads, require the use of a given amount of female material, placed on a support of adequate size in a predetermined position of the clothing or personal hygiene item, whose positioning occurs in a specific manufacturing step.

These aspects have a considerable effect on the manufacture of the final product and the relevant costs.

Our system overcomes the above problematic aspects and provides flexibility in terms of both operation and use, in addition to fulfilling the requirements of a considerable cost reduction.

The female material of the invention is not confined and not applied, but occupies and constitutes the support and operation surface of the device: it actually forms such surface.

A novel fastener system will be thus described hereafter in greater detail, which requires no reinforcement parts to preserve the integrity of the product over the mechanical fastening area.

Furthermore, the direct engagement of the male material as described above with the female material of the invention provides considerable resistances to tearing as well as the possibility of opening and closing the fastener device several times, without reducing its holding effect, which remains thus unchanged.

Hence, the inventor fulfills the object of obviating at least some of prior art problems and particularly the ones set out hereinbefore.

This object is fulfilled by a fastener device according to the features of claim 1, and by a clothing item according to the features of claim 9.

Further advantages may be obtained by the additional features of the dependent claims.

The invention will be now described with reference to the attached drawings in which:
- Figure 1 is a cross sectional view of a female surface of a fastener device;
- Figure 2 is an enlarged detail showing a male strap engaged with a female strap;
- Figure 3 is a perspective view of a fastener device with a male strap-like member, in which the female member forms the support layer of the finished item.

Referring to the annexed drawings, the releasable mechanical fastener device comprises a first male strap having a plurality of hook elements 11 which project out of at least one side 12 of the first strap 1.

The hook elements 11 may have conventional shapes ad sizes.

A second member 2 (female strap) is further provided, which is a laminate material 21, 22, comprising a polymer-based film 21 and a nonwoven fabric layer 22, preferably spun-bonded, attached to the polymer film 21.

The nonwoven fabric 22 and the polymer-based film 21 may be joined together by using cool melt and/or hot melt adhesives, heat sealing, ultrasounds.

The means for joining together the nonwoven fabric 22 and the film 21 are conventional and will not be further described.

The nonwoven fabric 22 of the second strap 2 has the peculiar characteristic of having a corrugated cross-sectional profile.

In the preferred embodiment, the corrugated profiles have a rectilinear extension, orthogonal to the longitudinal direction of the strap 1.

The corrugated cross-sectional profile may be obtained, for example, using a device as disclosed in US 6,499,640 B2 by the applicant hereof.

Thus, the corrugated profile adds elasticity to the female member to make the product better adaptable and to further counteract the tangential force (especially in clothing items and diapers) that tends to peel the male strap off by assisting the engagement of the hooking and enhancing the closing effect.

Preferably, the corrugated profile has a tip-to-tip pitch from about 1.8 mm to about 3.5 mm and a depth from 1.7 mm to 4.5 mm.

Preferably, the total basis weight of the second "strap" 2 is of 26 g/m2 to 50 g/m2.

More preferably, the basis weight of the second "strap" 2 is of 35 g/m2 to 45 g/m2.

In a possible embodiment, this laminate material has a water-vapor permeability, based on D6701 - 01 standard, of at least 500 (g H₂O/m²) /24 h, and an air permeability, based on ATICELCA MC 18-74 and TAPPI T 460 om-88 standards, below 100 min/ 100 cc of air.

The film 21 (of the second strap 2) may have an olefinic base material with fillers - such as the one disclosed in EP-B1-1,226,013 by the applicant hereof - or an olefinic and elastomeric base material with fillers - such as the one disclosed in WO 2005/051635 by the applicant hereof.

This solution is particularly interesting because it imparts a high elasticity to the second member and reduces the risk that the laminate material may be torn.

The spun-bonded nonwoven fabric strap 22 may be formed of polypropylene produced by traditional catalysis or by metallocene catalysis.

For example, the nonwoven fabric may be made using, as a starting material, the polypropylene currently sold by Innovene as 100-ZA25 and 100-ZA35 or the polypropylene currently sold by BASELL as HP651S and HM562S and finally by BOREALIS as HF420FB, HG420FB, HG455FB, HH420FB and HH450FB, or polypropylenes having similar characteristics (polypropylene homopolymers having MFRs from 25 g/10' to 35 g/10' and Melting Points from 160 °C to 165 °C).

Preferably, the fibers of the nonwoven fabric have a fineness of 1.5 to 2.5 deniers.

The above laminate material 21, 22 (comprising a polymer-based film 21 and a corrugated nonwoven fabric layer 22) may be used directly as a material for forming clothing and personal hygiene items.

For instance, for infant diapers and incontinence pads, the laminate material 21, 22 may form the support layer for the absorbent material

In this case, only the male straps 1 need to be applied to the product, as the surface of the product acts as a female member adapted to act as a base for engagement for the hook or mushroom elements 11 of the male straps 1.

In this case, it is obviously preferable for the laminate material to have the above air permeability and water-vapor permeability properties.

In clothing items and personal hygiene items, the use of a support structure in which the polymer film 21 is formed of a mixture of elastomers and/or olefins is particularly advantageous as it provides improved adjustment of fastener devices.

## Claims

1. A clothing or personal hygiene item, particularly an infant diaper or an incontinence pad, comprising a laminate (21, 22) having the function of a support layer for the absorbent material said laminate material (21, 22) comprising a polymer-based film (21) and a corrugated nonwoven fabric layer (22), said clothing or personal hygiene item comprising a releasable mechanical fastener device formed of at least one strap (1), having a plurality of hook or mushroom elements (11) which project out of at least one side (12) of said strap (1), said strap (1) being adapted to be engaged with said corrugated nonwoven fabric layer (22) of said laminate (21. 22) which occupies and constitutes the support and operation surface of the device.

2. A clothing or personal hygiene item as claimed in claim 1, wherein said corrugated profile of said nonwoven fabric (22) has a tip-to-tip pitch from 1.8 mm to 3.5 mm.

3. A clothing or personal hygiene item as claimed in claim 1 or 2, wherein said corrugated profile has a depth from 1. 7 mm to 4.5 mm.

4. A clothing or personal hygiene item as claimed in claim 1, 2 or 3, wherein the fibers of said nonwoven fabric (22) have a fineness from 1.5 deniers to 2.5 deniers.

5. A clothing or personal hygiene item as claimed in any one of claims 1 to 4, wherein said laminate material has a water-vapor permeability, based on ASTM D6701 - 01 standard, of at least 500 (g H2O/m²2)/24 h, and an air permeability, based on ATICELCA MC 18-74 and TAPPI T 460 om-88 standards, below 100 min/ 100 cc of air.

6. A clothing or personal hygiene item as claimed in any one of claims 1 to 5, wherein said laminate material (21, 22) has a total basis weight of 26 g/m2 to 50 g/m2.

7. A clothing or personal hygiene item as claimed in any one of claims 1 to 6, wherein said polymer-based film (21) is an olefin- and/or elastomer-based material with fillers.

## Patentansprüche

1. Kleidungsstück oder persönlicher Hygieneartikel, insbesondere Babywindel oder Inkontinenz-Tampon, aufweisend ein Laminat (21, 22), das die Funktion einer Halteschicht für das absorbierende Material hat, welches Laminat-Material (21, 22) eine polymerbasierte Folie (21) und eine wellige Faservlies-Schicht (22) aufweist, wobei das genannte Kleidungsstück oder der genannte persönlicher Hygieneartikel eine lösbare Verschlussvorrichtung mindestens eines Haltebands (1) hat, das eine Vielzahl von haken- oder pilzförmigen Elementen (11) aufweist, die an mindestens einer Seite (12) des Haltebands (1) vorstehen, welches Halteband (1) dazu ausgestaltet ist mit der genannten wellige Faservlies-Schicht (22) auf dem genannten Laminat (21, 22) verbunden zu werden, was die Halte- und Arbeitsoberfläche der Vorrichtung betrifft und ausmacht.

2. Kleidungsstück oder persönlicher Hygieneartikel nach Anspruch 1, wobei das genannte Wellenprofil des Faservlieses (22) eine Spitze-zu-Spitze Dicke von 1,8 mm bis 3,5 mm hat.

3. Kleidungsstück oder persönlicher Hygieneartikel nach Anspruch 1 oder 2, wobei das genannte Wellenprofil eine Tiefe von 1,7 mm bis 4,5 mm hat.

4. Kleidungsstück oder persönlicher Hygieneartikel nach Anspruch 1, 2 oder 3, wobei die Fasern des genannten Faservlieses (22) eine Feinheit von 1,5 Dernier bis 2,5 Dernier hat.

5. Kleidungsstück oder persönlicher Hygieneartikel nach einem der Ansprüche 1 bis 4, wobei das genante Laminat-Material eine auf dem ASTM D6701-01 Standard basierende Wasserdampf-Durchlässigkeit von mindestens 500 (g H₂O/m²)/24 h und eine auf dem ATICELCA MC 18-74 und TAPPI T 460 om-88 Standard basierende Luftdurchlässigkeit von weniger als 100 min/100 cc Luft aufweist.

6. Kleidungsstück oder persönlicher Hygieneartikel nach einem der Ansprüche 1 bis 5, wobei das genannte Laminat-Material (21, 22) ein Basisgesamtgewicht von 26 g/m² bis 50 g/m² hat.

7. Kleidungsstück oder persönlicher Hygieneartikel nach einem der Ansprüche 1 bis 6, wobei die genannte polymerbasierte Folie (21) ein olefin- und/oder elastomerbasiertes Material mit einer Füllmasse ist.

## Revendications

1. Vêtement ou article d'hygiène personnel, en particulier une couche d'enfant en bas âge ou un tampon d'incontinence, comprenant une bande (21, 22) ayant la fonction d'une bande d'appui pour le produit absorbant, ledit produit en bande (21, 22) comprenant un film à base de polymère (21) et une bande de tissu ondulé non-tissé (22), ledit vêtement ou article d'hygiène personnel comprenant un dispositif d'attache à ouverture mécanique rapide formé d'au moins une courroie (1) ayant une pluralité d'éléments en forme de crochet ou de champignon (11) qui projettent vers l'extérieur d'au moins un côté (12) de ladite courroie (1), ladite courroie (1) étant adaptée pour être engagée avec la couche de tissu ondulé non-tissé (22) de ladite bande (21, 22) qui occupe et constitue l'appui et la surface fonctionnelle du dispositif.

2. Vêtement ou article d'hygiène personnel selon les caractéristiques contenues dans la revendication 1, dans lequel ledit profil de tissu ondulé non-tissé (22) présente une distance bout-à-bout de 1,8 mm à 3,5 mm.

3. Vêtement ou article d'hygiène personnel selon les caractéristiques contenues dans la revendication 1 ou 2, dans lequel ledit profil ondulé a une profondeur de 1,7 mm à 4,5 mm.

4. Vêtement ou article d'hygiène personnel selon les caractéristiques contenues dans la revendication 1, 2 ou 3, où les fibres dudit tissu ondulé non-tissé (22) ont une épaisseur de 1,5 deniers à 2,5 deniers.

5. Vêtement ou article d'hygiène personnel selon les caractéristiques contenues dans l'une quelconque des revendications 1 à 4, où ledit produit en bande a une perméabilité à la vapeur d'eau, basée sur la norme ASTM D6701 - 01, d'au moins 500 (gH20/m2) /24 heures et une perméabilité aérienne, basée sur les normes ATICELCA MC 18-74 et TAPPI T 460 om-88, en-dessous de 100 min/100 cc d'air.

6. Vêtement ou article d'hygiène personnel selon les caractéristiques contenues dans l'une quelconque des revendications 1 à 5, où ledit produit en bande (21, 22) a un poids de base total de 26 g/m2 à 50 g/m2.

7. Vêtement ou article d'hygiène personnel selon les caractéristiques contenues dans l'une des revendications 1 à 6, où ledit film de base sur polymère (21) est un matériau à base d'élastomère et/ou d'oléfine avec des remplisseuses.
